

# UNITED STATES PATENT OFFICE.

AUGUSTE J. ROSSI, OF NIAGARA FALLS, NEW YORK, ASSIGNEE TO THE TITANIUM ALLOY MANUFACTURING COMPANY, OF NEW YORK, N. Y., A CORPORATION OF MAINE.

## METALLURGICAL METHOD.

1,104,317.

Specification of Letters Patent.

Patented July 21, 1914.

No Drawing.

Application filed April 10, 1914. Serial No. 831,052.

To all whom it may concern:

Be it known that I, AUGUSTE J. Rossi, a citizen of the United States, residing at Niagara Falls, in the county of Niagara and State of New York, have invented certain new and useful Improvements in Metallurgical Methods, of which the following is a specification.

My present invention relates to incorporation into iron, or its alloys, of titanium, or its compounds, and the objects of my invention comprise such incorporation in amounts sufficient for certain uses by manipulations more simple and economical, including lower temperatures, than heretofore.

Prior to my invention, in production of such products, by aid of carbon reduction, resort has been, as I believe, invariably had to such high temperatures, say 2500° C. at least, or much higher, as can, with industrial practicability, be developed only in electric furnaces as per, among my Letters Patent, No. 609,466, dated August 23, 1898 for "alloy of iron and process of producing it"; also No. 1,039,672, dated September 24, 1912, or, as can be developed, by aluminum reduction of titanic oxid as per Reissue No. 12,674, dated March 17, 1908. Such relatively high temperatures still appear indispensable in production of alloys containing such relatively high percentages of titanium, or its desired compounds, including its carbid, as say 10% or more, but I have discovered that in cases in which percentages as low as say 5 to 1 per cent. or less suffice for certain purposes, as for example in purification, or in recarburizing, of steel or other metals, as per among my Patents, Nos. 1,056,125, dated March 18, 1913, or No. 1,003,805, dated September 19, 1911, such lower alloys, or compounds, are producible, and sometimes more advantageously, under conditions and by procedures requiring no higher temperatures than those of the open hearth (1600° to 1700° C.), or the blast furnace (1510° C.) or even lower; provided there be present, during some stage of the operation, enough manganese, *i. e.* manganese in elemental, metallic state.

If so-called titaniferous iron, or ilmenite, ores, as for example those from the neighborhood of Baie St. Paul, Canada, containing often, as high as 36.88% to 40% of

titanic acid and about 50% oxids of iron, be smelted, as per usual approved blast furnace practice, *i. e.* by aid of carbon and fluxes, as for instance, per my Patent 486,941, dated November 29, 1892, the pig will contain no, or not to exceed an insignificant fraction of one per cent., of, titanic material in any form, such constituents of the ore proving, under such conditions, so refractory as to pass off in the slag. But, if, as per my present invention, manganese, in sufficient quantity, be, by any means, made present in the charge, during such operation at the said usual, relatively low, temperatures, then, as I have discovered, the result is pig containing important percentages, say 5% or 1%, or more or less, of titanium, or its carbid, or both. I have also discovered that if the manganese, so employed, be derived from its oxid, introduced as such, the pig will contain a much higher percentage of that metal also than if titanic oxid were absent. Extended research and consideration have hitherto failed to disclose an altogether satisfactory explanation for these unexpected phenomena, but repeated tests establish that presence of enough molten manganese, particularly if in nascent state, insures reduction of titanic oxid at much lower than hitherto deemed requisite temperatures, and that the occurrence of  $TiO_2$  reduction serves to increase reduction of oxid manganese if present.

In considering the merits of my present invention it is also to be noted that iron ores containing enough titanic constituents to be distinguishable as "titaniferous," say not less than 3%, are almost invariably found in nature not to contain above 1% of oxid of manganese, in fact generally only a few hundredths, or tenths, of one per cent. On the other hand, the reverse is, so far as I know, true of so-called "manganiferous ores," the which, containing more than 1% of oxid of manganese, appear, in nature, to be devoid of titanic oxid, or containing not to exceed insignificantly small fractions of 1% thereof. I therefore infer that the results of my invention have, prior thereto, been unattained, and are substantially unattainable by reduction, or smelting, of unadmixed, natural, ores.

In explanation and support of the above, I refer to some of my operations as follows,

viz:—I selected a titaniferous iron ore of the following composition, viz:—iron oxid 50.14,  $TiO_2$  36.88,  $SiO_2$  2.92,  $MgO$  3.27,  $CaO$  0.50,  $Al_2O_3$  4.80,  $MnO_2$  0.21. Four lots of 5 this ore were smelted at different times in a blast furnace according to usual, approved, blast furnace practice, and resulting pigs obtained, which, by analysis, were indicated to have contained of titanic substances, in 10 whatever form, no more than the following, viz:—Lot No. 1, 0.03 titanium; lot No. 2, 0.05; lot No. 3, 0.025; lot No. 4, 0.000. I thereafter mixed with the same ore oxid of manganese ( $MnO_2$ ) in the ratio of 100 parts 15 of ore to 30 of said oxid, and smelting the mixture, as before, obtained a pig containing, by analyses, titanium 1.94, and manganese 2.56, carbon 4.16. From another similar test with the same ore in which I ad- 20 mixed therewith 40 parts of  $MnO_2$ , I obtained a pig analyzing titanium 2.05 and over, and manganese 3.02. I have conducted other similar operations in which the additions of manganese oxid were less in pro- 25 portion to titanic oxid, and obtained pig metals analyzing from 0.79 to 0.9 of titanium existing as such, or as compounds there- of in such pigs.

My invention is practised by incorporating 30 into any usual approved, open hearth, or blast furnace, or other, charge comprising titaniferous iron ore, fluxes and carbon, oxid of manganese, as, for example, preferably, by admixture with the charge of man- 35 ganiferous iron ore, or ore containing sufficient oxid of manganese, the essential being to secure presence of sufficient molten manganese, preferably nascent, during the opera- 40 tion.

The charge is, of course, during the opera- 45 tion, heated, but, preferably, not to exceed the temperatures sufficient to reduce oxids of iron or manganese as in usual blast, or open hearth, furnace practice, say 1510° C. to not to exceed 1700° C., but my results are attainable at temperatures even lower.

The proportions of manganese or its com- 50 pounds employed will be readily determined according to the requirements of each case by those skilled in the art. They will de- 55 pend, to an extent, on the proportion of titanic oxid present, and the per cent. of metallic titanium, or its compounds, desired, or feasible to incorporate, in the resulting product.

My researches have, up to the present, in- 60 dicated that in no operation of my method can any important, or practically useful, amount of titanium, or its carbid, be ex- 65 pected in the final product, unless the titaniferous iron ore employed contain not less than 3% of titanic oxid, and there be in the charge, oxid of manganese in quantity not less than equal to 10% of the titanic oxid present, or, in lieu of said oxid of manga-

nese, there be present manganese represent- 70 ing the metallic resultant, to be expected from reduction of said proportion of its said oxid relatively to the titanic oxid. However, excess of either of these minimums, neither prevents the desired result, nor is, I believe, detrimental, unless for economical, or other, 75 reasons.

Under the conditions specified, I have been unable, as yet, to incorporate, in the final product, more than say 5% of titanium, or its compounds, notwithstanding presence of sufficient carbon and much more than sufficient oxid of titanium and manganese. It goes without saying that in all cases car- 80 bon should be supplied as usual in quantity sufficient to reduce the iron oxids of the charge, and enough to reduce as much of the oxids of titanium and manganese as is fea- 85 sible under the temperatures employed as aforesaid, subject to the above limitations.

After the reactions have proceeded as far as possible, or desired, the resulting molten metal is withdrawn and cast as usual, and will be found to contain, in addition to iron, manganese, and carbon, from say less than one to five per cent. of titanium, or say its carbid, or both, depending, in part, on the proportions of titanic oxid, carbon and manganese in the charge; and on the tempera- 90 tures.

The product is useful for many purposes, including purification, or recarburization, of metals, or their alloys. Its production, as aforesaid, is, as will be appreciated, more economical than by previous methods of incorporating into ferro metals titanium or its compounds derived from titanic oxid, and my method is also particularly valuable because utilizable in, and as part of, usual 95 blast furnace or open hearth operations with titaniferous iron ores.

Having now described my invention what I claim as new and desire to secure by Letters Patent is the following:

1. The metallurgical method which com- 100 prises bringing together carbon, titaniferous iron ore containing not less than 3% con- 105 tent of titanic oxid, and oxid of manganese in quantity not less than 10% of said titanic oxid, and melting them together at tempera- 110 ture below 1700° C.

2. The metallurgical method which com- 115 prises bringing together carbon, titaniferous iron ore containing not less than 3% con- 120 tent of titanic oxid, and manganeseiferous iron ore, and melting them together at tempera- 125 ture below 1700° C.

3. The metallurgical method which com- 125 prises bringing together carbon, titanic oxid, and oxid of manganese in quantity not less than 10% of said titanic oxid, and melting them together at temperature below 1700° C.

4. The metallurgical method which com- 130 prises bringing together carbon, titaniferous

iron ore, and manganiferous iron ore, and melting them together at temperature below 1700° C.

5. The metallurgical method which comprises bringing together carbon, titanic oxid, and manganiferous iron ore, and melting them together at temperature below 1700° C.

6. The metallurgical method which comprises bringing together carbon, titaniferous iron ore containing not less than 3% content of titanic oxid, and oxid of manganese in quantity not less than 10% of said titanic oxid, and melting them together.

7. The metallurgical method which comprises bringing together carbon, titaniferous iron ore containing not less than 3% content of titanic oxid, and manganiferous iron ore, and melting them together.

8. The metallurgical method which comprises bringing together carbon, titanic oxid, and oxid of manganese in quantity not less than 10% of said titanic oxid, and melting them together.

9. The metallurgical method which comprises bringing together carbon, titaniferous iron ore, and manganiferous iron ore, and melting them together.

10. The metallurgical method which comprises bringing together carbon, titanic oxid, and manganiferous iron ore, and melting them together.

11. In the incorporation of a titanic substance into a ferro-metal, the step which consists in supplying molten manganese to a charge containing such metal, carbon, and titanic oxid.

12. In the incorporation of a titanic substance into a ferro-metal, the step which consists in supplying to a charge containing

such metal, carbon, and titanic oxid, molten manganese derived by reduction of a quantity of its oxid not less than 10% of said titanic oxid.

13. In the incorporation of a titanic substance into a ferro-metal, the step which consists in supplying molten manganese to a charge maintained throughout the operation at temperatures not to exceed 1700° C. and containing such ferro-metal, carbon, and titanic oxid.

14. In the incorporation of a titanic substance into a ferro-metal, the step which consists in supplying to a charge maintained throughout the operation at temperatures not to exceed 1700° C. and containing such metal, carbon, and titanic oxid, molten manganese derived by reduction of a quantity of its oxid not less than 10% of said titanic oxid.

15. As a new article of manufacture, the ternary alloy of iron, titanium, and manganese.

16. As a new article of manufacture, an alloy, or compound, containing preponderance of iron, titanium not to exceed 5%, manganese, and carbon.

17. As a new article of manufacture, an alloy, or compound, containing iron, titanium, manganese, and carbon.

18. As a new article of manufacture, an alloy, or compound, containing carbon, iron, titanium, and manganese not less than one per cent.

AUGUSTE J. ROSSI.

Witnesses:

PHILIP C. REH,  
ALFRED R. CONANT.